

# UNITED STATES PATENT OFFICE.

JOHN P. WRIGHT, OF NEWARK, DELAWARE.

## COMPOSITE BOARD.

1,303,753.

Specification of Letters Patent. Patented May 13, 1919.

No Drawing.

Application filed February 26, 1918. Serial No. 80,710.

To all whom it may concern:

Be it known that I, JOHN P. WRIGHT, a citizen of the United States, residing at Newark, in the county of Newcastle and 5 State of Delaware, have invented certain new and useful Improvements in Composite Board, of which the following is a specification.

My invention relates to an improvement 10 in the art of manufacturing composite board, or articles therefrom, the board possessing strength, rigidity and stability.

Hitherto there has been made a composite board in which bakelite or similar material 15 used as a binder was employed merely as a superficial coating for the surface of the layers of the web or paper fabric, and the objection to this treatment has been that there are intermediate layers of paper or 20 fabric, and in fact, the inside fibers of the layers are not coated and consequently the entire finished product is not thoroughly homogeneous and alike throughout.

My present invention comprises laminated 25 layers of material, such as paper, or duck, saturated with a substance commercially known as bakelite, or similar material possessing the same general characteristics, and subjected to suitable heat and pressure, 30 whereby a homogeneous product results, possessing the qualities of rigidity and stability, being water-proof, and having insulating qualities, and capable of being used for various purposes, and made up in different forms, such as gears, tubes, or in flat 35 sheets capable of being worked over into various articles of manufacture requiring some or all of the qualifications mentioned.

In order to prepare a card-board having 40 the foregoing characteristics, I propose to proceed substantially as follows: I take an unsized absorbent paper, preferably especially prepared for the purpose. Each sheet is saturated with bakelite or material having 45 similar characteristics, thus making a separate sheet or unit of the character of the entire product, and the product consequently, although made of laminated sheets, becomes in reality a homogeneous composite. 50 The material used may be a liquid condensation product of phenols and formaldehyde of such character that it is capable of transformation under the action of heat into an insoluble and infusible body.

Obviously other substances that have the 55 ability to harden under heat, as, for instance,

some varnishes that may exist or may be developed, might be used in my method of saturation as distinguished from mere coating of layers, producing possibly even a better product than with the use of bakelite.

For this purpose, I may use either a liquid condensation product of the character described, or a solution of the same in alcohol or other appropriate solvent. This layer is 60 permitted to dry somewhat, when a second sheet of paper is superposed upon the first, and similarly treated, or the several layers may be saturated and preferably dried before being superposed. The desired number 65 of sheets having been assembled, the composite article is compacted by pressure, with or without the aid of heat. Heat is now applied only to affect the transformation of the condensation product into an insoluble, infusible body. The heat may be applied during the operation of compressing or compacting the composite body, or at a subsequent stage of the process; or it may be 70 applied partly during the compressing operation, and continued during subsequent stages.

The compressed product may be heated gradually in an oven, starting at relatively low temperatures, say 40° C. to 80° C. and 75 gradually increasing to higher temperatures, for instance 100° C. to 140° C. the increase in temperature being so gradual as to avoid the formation of blisters or other irregularities.

Instead of superposing a number of separate sheets, the liquid condensation product may be applied to a continuous sheet or web, which may then be rolled upon itself in the form of a tube, suitable mechanical devices 80 being used for this purpose. The tubes thus formed may then be cut and straightened into composite sheets before hardening, according to the use for which they are intended.

Likewise this same process is applicable to tubes to be used as such, in which event the saturated superimposed layers formed by winding or otherwise as the case may be are hardened before they are available for commercial use.

The condensation products for use as above may be mixed with pigments, or dyes, or they may be used in conjunction with a certain proportion of resinous material. 105 The length of time the heat is applied is dependent entirely on the thickness of the ma-

terial. The longer the product is left under conditions of heat and pressure, the more brittle it becomes.

Where canvas is used, the best quality of canvas duck is preferred, and either the sheets or tubes could be made of the paper or canvas duck, as desired. The completed product is absolutely water-proof throughout, that is to say every fiber in it all the way through is waterproof, and the result is that the product can be used anywhere where hard rubber is used, as the product will keep out moisture, and is practically as waterproof as rubber.

In addition to the use of an especially prepared unsized absorbent paper, impregnation could be accomplished by any of the ordinary approved methods, for instance by the vacuum system, by forcing in under pressure or by any other method, and consequently it is not my desire to be limited to the exact method of saturation or impregnation hereinbefore cited, this invention contemplating the broad idea of saturation producing homogeneity.

It is also probable that the results might be obtained by using a solvent such as alcohol, as for instance a very thick varnish would not saturate a sheet of paper or fabric, unless, perhaps it is thinned down with some suitable solvent.

This product is consequently especially adapted to use in wireless installations, where a material is necessary which will not absorb moisture.

This material is easily machined, fashioned, threaded, and toothed as occasion may

require in its application to use in various industries.

I claim:

1. A composite product composed of laminations of fibrous material, each lamination being saturated throughout with approximate uniformity, with a phenolic condensation product, and the whole being subjected to sufficient pressure and heat to form an approximately homogeneous product.

2. A composite product composed of laminations of paper or the like, each lamination being saturated throughout with approximate uniformity, with a phenolic condensing product, the whole being subjected to sufficient pressure and heat to form an approximately homogeneous product.

3. A composite product composed of laminations of paper or the like, each lamination being saturated throughout with approximate uniformity with a substance commercially known as or having the qualities of bakelite, and the whole being subjected to sufficient pressure and heat to form approximately homogeneous product.

4. The method of producing a composite product which consists in saturating an absorbent medium with a phenolic condensation product, then drying each until the solvent is entirely dried out of the liquid, then piling said absorbent medium into layers and applying heat and pressure to first soften and then harden the phenolic condensation product with which each absorbent layer is saturated.

In testimony whereof I affix my signature.

JOHN P. WRIGHT.